

## UNITED STATES PATENT OFFICE

2,463,010

## METHOD OF REDUCING CORROSION

John O. Almen, Royal Oak, Mich., assignor to  
General Motors Corporation, Detroit, Mich., a  
corporation of Delaware

No Drawing. Application January 5, 1944,  
Serial No. 517,102

3 Claims. (Cl. 29—148)

1

Shot peening or blasting a surface with smooth steel balls for compressively stressing the skin of a metal article increases materially resistance to fatigue failure. I have discovered that proper peening can be effected for the purpose of resisting corrosion of several kinds. For example, a magnesium strip one-sixteenth of an inch in thickness stressed by bending will fail by stress corrosion in approximately two minutes' time when immersed in a salt solution. On the other hand the same specimen will endure indefinitely after the surface has been compressively stressed by light shot peening in the manner to be described.

Magnesium or other similar metals when closely fitted to a dissimilar metal, such as iron, are likely to corrode badly. Corrosion which occurs between bolted surfaces, on splines, press fits and other like closely fitted parts is known under the general name of fretting corrosion. Such corrosion is retarded and its penetration reduced by compressively prestressing the surface. Stress corrosion is severe in magnesium and its avoidance is of special importance in aircraft construction largely comprised of magnesium metals in critical parts.

Rapid electrolytic corrosion occurs on such metals as aluminum, magnesium, etc., when iron dust is retained on the surface of the metal from shot blasting. Such corrosion occurs on exposed surfaces particularly when immersed in salt solutions although it will occur in the atmosphere particularly in damp weather, such as rusting of steel parts.

Stress corrosion is the more rapid attack of normal atmospheric corrosion. The penetration is rapid, presumably because when a tension stress is present the gaps formed by corrosive severance of the bonds of adjacent particles will be opened permitting corrosion to progress deeply into the material. When the material is compressively stressed there is a tendency for the gaps to be closed, and therefore corrosion does not progress deeply into the material.

Fretting corrosion is that which occurs between tightly fitted parts whether of the same metal or of dissimilar metals or, in fact, between metals and organic materials such as plastics, paper, etc. This corrosion results from very small motions between the tightly fitted parts. It may fundamentally be an electrolytic action since we are told that all corrosion is electrolytic, but electrolytic action may occur without the presence of dissimilar metals. Burns of the Bell Laboratories states that electrolytic action may occur in a

2

metal between regions of dissimilar stress. Fretting corrosion, therefore, is not dependent on the contamination due to shot peening whether the fretting corrosion occurs between similar or dissimilar metals.

Compressively prestressing the surface of parts subject to corrosion damage has proved itself highly effective. However, care must be exercised to see that the metal surface to be compressed is free from contact with a dissimilar metal during the prestressing operation including dust or flake particles from the shot which tend to accumulate at the shot blasting station and to settle on articles being operated upon and under the hammering to be embedded in and to contaminate the metal surface. Thus iron dust from steel shot would contaminate the surface of a magnesium article and must be removed or prevented from adhering in order to avoid subsequent electrolytic action between the dissimilar metals which electrolytic action would undo the effect of prestressing in reducing corrosion.

Magnesium and similar materials corrode very rapidly when stressed in tension and less rapidly when unstressed. The object of compressive prestressing is to place a thin surface layer of the material in a state of compression even though underlying layers are stressed in tension.

To accomplish the result, I have used the expedient of coating the surface of the article to be treated with a strong paint or lacquer and then after the coating has dried and set, peening through the coating. A strongly adherent and elastic paint is required to avoid flaking during the peening operation but the coating should be thin so as not to unduly cushion the impact of the shot. Thus the impacts are transmitted to the metal surface by means of a nonmetallic agency and the surface is maintained free from contamination. Once the surface has been densified the paint, if desired, can be removed and at any rate the magnesium may be joined or press fitted to an iron part without fear of serious corrosion problems. As an alternative to accomplish the same result in the absence of contact between dissimilar metals, it is proposed to use smooth shot of a nonmetallic material, such as glass or a relatively strong plastic. Glass shot has been found to be satisfactory for this purpose.

In my study of the problem I have noted resistance to other forms of corrosion results from shot peening. Fretting corrosion has been greatly reduced by peening with iron shot. This has been observed on numerous steel specimens. In this case superficial corrosion may be increased

due to the surface roughness of the peened specimen but penetration of corrosion is apparently greatly reduced. Similar results have been obtained in fretting corrosion between dissimilar metals in airplane engines.

In addition to shot peening, the results described above may be obtained by other prestressing means such as rolling with small rollers or balls. It is only necessary that the surface of the metal be stressed in compression.

I claim:

1. The method of reducing surface corrosion between tightly fitted parts of dissimilar metals, comprising subjecting one of the parts, before they are tightly fitted, to a conditioning treatment which includes precrating the joint surface with a thin elastic film capable of transmitting impact therethrough and incapable of electrolytic action with the material of said surface and compressively stressing the surface beneath said film by repetitive blows of an impacting body against the film covered skin of the joint surface which precompresses the film covered skin of the joint surface and thereafter tightly fitting together said parts with the joint surfaces of one in contact with the precompressed skin of the joint surface of the other.

2. The method of decreasing the tendency toward surface corrosion in articles containing a magnesium metal, including applying on the surface to be protected, a coating of strongly adherent and elastic paint, allowing the paint to set and then peening the metal through the coating to stress the surface of the metal in compression.

3. The method of prestressing in compression the surface of an article formed of largely magnesium including peening said surface by blasting the same with nonmetallic smooth and uniformly spherical shot.

JOHN O. ALMEN.

#### REFERENCES CITED

The following references are of record in the file of this patent:

#### UNITED STATES PATENTS

|    | Number    | Name     | Date           |
|----|-----------|----------|----------------|
| 15 | 326,469   | Youngs   | Sept. 15, 1885 |
|    | 489,642   | Reich    | Jan. 10, 1893  |
|    | 1,433,213 | Lowell   | Oct. 24, 1922  |
|    | 2,043,481 | Krissiep | June 9, 1936   |
|    | 2,058,841 | Thomson  | Oct. 27, 1936  |
|    | 2,149,253 | Cooper   | Mar. 7, 1939   |
| 20 | 2,185,262 | Lupo     | Jan. 2, 1940   |
|    | 2,208,732 | Powell   | July 23, 1940  |
|    | 2,234,491 | Hayden   | Mar. 11, 1941  |
|    | 2,349,395 | Zublin   | May 23, 1944   |

#### FOREIGN PATENTS

|  | Number  | Country       | Date         |
|--|---------|---------------|--------------|
|  | 284,313 | Great Britain | Mar. 1, 1928 |
|  | 288,637 | Germany       | Nov. 9, 1915 |

#### OTHER REFERENCES

30 Pub., "The Technology of Magnesium and Its Alloys," F. A. Hughes & Co. Ltd., London, 1940, pages 231, 233.

35 Metals Handbook, 1939 ed., Am. Society for Metals, Cleveland, Ohio, page 1614.